



US008778098B2

(12) **United States Patent**  
**Pandey**

(10) **Patent No.:** **US 8,778,098 B2**  
(45) **Date of Patent:** **\*Jul. 15, 2014**

(54) **METHOD FOR PRODUCING HIGH STRENGTH ALUMINUM ALLOY POWDER CONTAINING L1<sub>2</sub> INTERMETALLIC DISPERSOIDS**

(75) Inventor: **Awadh B. Pandey**, Jupiter, FL (US)

(73) Assignee: **United Technologies Corporation**, Hartford, CT (US)

(\*) Notice: Subject to any disclaimer, the term of this patent is extended or adjusted under 35 U.S.C. 154(b) by 259 days.

This patent is subject to a terminal disclaimer.

(21) Appl. No.: **12/316,047**

(22) Filed: **Dec. 9, 2008**

(65) **Prior Publication Data**

US 2010/0143185 A1 Jun. 10, 2010

(51) **Int. Cl.**

*C22C 21/02* (2006.01)  
*C22C 1/04* (2006.01)  
*B22F 9/08* (2006.01)  
*B22F 3/20* (2006.01)  
*C22C 21/00* (2006.01)  
*C22F 1/04* (2006.01)

(52) **U.S. Cl.**

CPC ..... *C22C 21/00* (2013.01); *B22F 9/082* (2013.01); *C22F 1/04* (2013.01); *C22C 1/0416* (2013.01)  
USPC ..... **148/438**; 75/249; 75/339; 148/689; 419/67

(58) **Field of Classification Search**

CPC ..... B22F 3/20; B22F 3/227  
USPC ..... 148/415-418, 437-440, 549-552;  
420/528-554; 75/338-341

See application file for complete search history.

(56)

**References Cited**

U.S. PATENT DOCUMENTS

|             |         |                    |
|-------------|---------|--------------------|
| 3,619,181 A | 11/1971 | Willey et al.      |
| 3,816,080 A | 6/1974  | Bomford et al.     |
| 4,041,123 A | 8/1977  | Lange et al.       |
| 4,259,112 A | 3/1981  | Dolowy, Jr. et al. |
| 4,463,058 A | 7/1984  | Hood et al.        |
| 4,469,537 A | 9/1984  | Ashton et al.      |
| 4,499,048 A | 2/1985  | Hanejko            |
| 4,597,792 A | 7/1986  | Webster            |
| 4,626,294 A | 12/1986 | Sanders, Jr.       |

(Continued)

FOREIGN PATENT DOCUMENTS

|    |             |        |
|----|-------------|--------|
| CN | 1436870 A   | 8/2003 |
| CN | 101205578 A | 6/2008 |

(Continued)

OTHER PUBLICATIONS

A. Unal (Uenal), D.D. Leon, T.B. Gurganus, G.J. Hilderman, "Production of Aluminum and Aluminum-Alloy Powder," vol. 7: Powder Metal Technologies and Applications, ASM Handbooks Online, ASM International, 2002, 26 pages total, orig. published in 1998 in pp. 148-159 in vol. 7 of ASM Handbook by ASM International.\*

(Continued)

*Primary Examiner* — Scott Kastler

*Assistant Examiner* — Vanessa Luk

(74) *Attorney, Agent, or Firm* — Kinney & Lange, P.A.

(57) **ABSTRACT**

A method for producing high strength aluminum alloy powder containing L<sub>1</sub><sub>2</sub> intermetallic dispersoids uses high pressure gas atomization to effect cooling rates in excess of 10<sup>30</sup> C./second.

**7 Claims, 9 Drawing Sheets**



(56)

## References Cited

## U.S. PATENT DOCUMENTS

|                |         |                    |                   |         |                   |         |
|----------------|---------|--------------------|-------------------|---------|-------------------|---------|
| 4,647,321 A    | 3/1987  | Adam               | 7,883,590 B1 *    | 2/2011  | Pandey .....      | 148/439 |
| 4,661,172 A    | 4/1987  | Skinner et al.     | 7,909,947 B2 *    | 3/2011  | Pandey .....      | 148/439 |
| 4,667,497 A    | 5/1987  | Oslin et al.       | 8,002,912 B2 *    | 8/2011  | Pandey .....      | 148/437 |
| 4,689,090 A    | 8/1987  | Sawtell et al.     | 8,017,072 B2 *    | 9/2011  | Pandey .....      | 420/550 |
| 4,710,246 A    | 12/1987 | Le Caer et al.     | 2001/0054247 A1   | 12/2001 | Stall et al.      |         |
| 4,713,216 A    | 12/1987 | Higashi et al.     | 2003/0192627 A1   | 10/2003 | Lee et al.        |         |
| 4,755,221 A    | 7/1988  | Paliwal et al.     | 2004/0046402 A1   | 3/2004  | Winardi           |         |
| 4,832,741 A    | 5/1989  | Couper             | 2004/0055671 A1 * | 3/2004  | Olson et al. .... | 148/561 |
| 4,834,810 A    | 5/1989  | Benn et al.        | 2004/0089382 A1   | 5/2004  | Senkov et al.     |         |
| 4,834,942 A    | 5/1989  | Frazier et al.     | 2004/0170522 A1   | 9/2004  | Watson            |         |
| 4,853,178 A    | 8/1989  | Oslin              | 2004/0191111 A1   | 9/2004  | Nie et al.        |         |
| 4,865,806 A    | 9/1989  | Skibo et al.       | 2005/0013725 A1   | 1/2005  | Hsiao             |         |
| 4,874,440 A    | 10/1989 | Sawtell et al.     | 2005/0147520 A1   | 7/2005  | Canzona           |         |
| 4,915,605 A    | 4/1990  | Chan et al.        | 2006/0011272 A1   | 1/2006  | Lin et al.        |         |
| 4,923,532 A    | 5/1990  | Zedalis et al.     | 2006/0093512 A1   | 5/2006  | Pandey            |         |
| 4,927,470 A    | 5/1990  | Cho                | 2006/0172073 A1   | 8/2006  | Groza et al.      |         |
| 4,933,140 A    | 6/1990  | Oslin              | 2006/0269437 A1   | 11/2006 | Pandey            |         |
| 4,946,517 A    | 8/1990  | Cho                | 2007/0048167 A1   | 3/2007  | Yano              |         |
| 4,964,927 A    | 10/1990 | Shiflet et al.     | 2007/0062669 A1   | 3/2007  | Song et al.       |         |
| 4,988,464 A    | 1/1991  | Riley              | 2008/0066833 A1   | 3/2008  | Lin et al.        |         |
| 5,032,352 A    | 7/1991  | Meeks et al.       |                   |         |                   |         |
| 5,053,084 A    | 10/1991 | Masumoto et al.    | EP 0 584 596 A2   | 3/1994  |                   |         |
| 5,055,257 A    | 10/1991 | Chakrabarti et al. | EP 1 111 079 A1   | 6/2001  |                   |         |
| 5,059,390 A    | 10/1991 | Burleigh et al.    | EP 1 249 303 A1   | 10/2002 |                   |         |
| 5,066,342 A    | 11/1991 | Rioja et al.       | EP 1 170 394 B1   | 4/2004  |                   |         |
| 5,076,340 A    | 12/1991 | Bruski et al.      | EP 1 439 239 A1   | 7/2004  |                   |         |
| 5,076,865 A    | 12/1991 | Hashimoto et al.   | EP 1 471 157 A1   | 10/2004 |                   |         |
| 5,130,209 A    | 7/1992  | Das et al.         | EP 1 111 078 B1   | 9/2006  |                   |         |
| 5,133,931 A    | 7/1992  | Cho                | EP 1 728 881 A2   | 12/2006 |                   |         |
| 5,198,045 A    | 3/1993  | Cho et al.         | EP 1 788 102 A1   | 5/2007  |                   |         |
| 5,211,910 A    | 5/1993  | Pickens et al.     | FR 2110452 A1     | 10/2009 |                   |         |
| 5,226,983 A    | 7/1993  | Skinner et al.     | JP 2843754 A1     | 2/2004  |                   |         |
| 5,256,215 A    | 10/1993 | Horimura           | JP 04218638 A     | 8/1992  |                   |         |
| 5,308,410 A    | 5/1994  | Horimura et al.    | JP 9104940 A      | 4/1997  |                   |         |
| 5,312,494 A    | 5/1994  | Horimura et al.    | JP 9279284 A      | 10/1997 |                   |         |
| 5,318,641 A    | 6/1994  | Masumoto et al.    | JP 11156584 A     | 6/1999  |                   |         |
| 5,397,403 A    | 3/1995  | Horimura et al.    | JP 2000119786 A   | 4/2000  |                   |         |
| 5,458,700 A    | 10/1995 | Masumoto et al.    | JP 2001038442 A   | 2/2001  |                   |         |
| 5,462,712 A    | 10/1995 | Langan et al.      | JP 2006248372 A   | 9/2006  |                   |         |
| 5,480,470 A    | 1/1996  | Miller et al.      | JP 2007188878 A   | 7/2007  |                   |         |
| 5,532,069 A    | 7/1996  | Masumoto et al.    | KR 20040067608 A  | 7/2004  |                   |         |
| 5,597,529 A    | 1/1997  | Tack               | WO 90 02620 A1    | 3/1990  |                   |         |
| 5,620,652 A    | 4/1997  | Tack et al.        | WO 91 10755 A2    | 7/1991  |                   |         |
| 5,624,632 A    | 4/1997  | Baumann et al.     | WO 9111540 A1     | 8/1991  |                   |         |
| 5,882,449 A    | 3/1999  | Waldron et al.     | WO 9532074 A2     | 11/1995 |                   |         |
| 6,139,653 A    | 10/2000 | Fernandes et al.   | WO 96/10099 A1    | 4/1996  |                   |         |
| 6,149,737 A    | 11/2000 | Hattori et al.     | WO 9833947 A1     | 8/1998  |                   |         |
| 6,248,453 B1   | 6/2001  | Watson             | WO 00 37696 A1    | 6/2000  |                   |         |
| 6,254,704 B1   | 7/2001  | Laul et al.        | WO 0112868 A1     | 2/2001  |                   |         |
| 6,258,318 B1   | 7/2001  | Lenczowski et al.  | WO 02 29139 A2    | 4/2002  |                   |         |
| 6,309,594 B1   | 10/2001 | Meeks, III et al.  | WO 03 052154 A1   | 6/2003  |                   |         |
| 6,312,643 B1   | 11/2001 | Upadhyaya et al.   | WO 03085145 A2    | 10/2003 |                   |         |
| 6,315,948 B1   | 11/2001 | Lenczowski et al.  | WO 03085146 A1    | 10/2003 |                   |         |
| 6,331,218 B1   | 12/2001 | Inoue et al.       | WO 03 104505 A2   | 12/2003 |                   |         |
| 6,355,209 B1   | 3/2002  | Dilmore et al.     | WO 2004 005562 A2 | 1/2004  |                   |         |
| 6,368,427 B1   | 4/2002  | Sigworth           | WO 2004046402 A2  | 6/2004  |                   |         |
| 6,506,503 B1   | 1/2003  | Mergen et al.      | WO 2005 045080 A1 | 5/2005  |                   |         |
| 6,517,954 B1   | 2/2003  | Mergen et al.      | WO 2005047554 A1  | 5/2005  |                   |         |
| 6,524,410 B1   | 2/2003  | Kramer et al.      |                   |         |                   |         |
| 6,531,004 B1   | 3/2003  | Lenczowski et al.  |                   |         |                   |         |
| 6,562,154 B1   | 5/2003  | Rioja et al.       |                   |         |                   |         |
| 6,630,008 B1   | 10/2003 | Meeks, III et al.  |                   |         |                   |         |
| 6,702,982 B1   | 3/2004  | Chin et al.        |                   |         |                   |         |
| 6,902,699 B2   | 6/2005  | Fritzemeier et al. |                   |         |                   |         |
| 6,918,970 B2   | 7/2005  | Lee et al.         |                   |         |                   |         |
| 6,974,510 B2   | 12/2005 | Watson             |                   |         |                   |         |
| 7,048,815 B2   | 5/2006  | Senkov et al.      |                   |         |                   |         |
| 7,097,807 B1   | 8/2006  | Meeks, III et al.  |                   |         |                   |         |
| 7,241,328 B2   | 7/2007  | Keener             |                   |         |                   |         |
| 7,344,675 B2   | 3/2008  | Van Daam et al.    |                   |         |                   |         |
| 7,811,395 B2 * | 10/2010 | Pandey .....       |                   |         |                   |         |
| 7,871,477 B2 * | 1/2011  | Pandey .....       |                   |         |                   |         |
| 7,875,131 B2 * | 1/2011  | Pandey .....       |                   |         |                   |         |
| 7,875,133 B2 * | 1/2011  | Pandey .....       |                   |         |                   |         |
| 7,879,162 B2 * | 2/2011  | Pandey .....       |                   |         |                   |         |

## FOREIGN PATENT DOCUMENTS

|                   |         |
|-------------------|---------|
| EP 0 584 596 A2   | 3/1994  |
| EP 1 111 079 A1   | 6/2001  |
| EP 1 249 303 A1   | 10/2002 |
| EP 1 170 394 B1   | 4/2004  |
| EP 1 439 239 A1   | 7/2004  |
| EP 1 471 157 A1   | 10/2004 |
| EP 1 111 078 B1   | 9/2006  |
| EP 1 728 881 A2   | 12/2006 |
| EP 1 788 102 A1   | 5/2007  |
| EP 2110452 A1     | 10/2009 |
| FR 2843754 A1     | 2/2004  |
| JP 04218638 A     | 8/1992  |
| JP 9104940 A      | 4/1997  |
| JP 9279284 A      | 10/1997 |
| JP 11156584 A     | 6/1999  |
| JP 2000119786 A   | 4/2000  |
| JP 2001038442 A   | 2/2001  |
| JP 2006248372 A   | 9/2006  |
| JP 2007188878 A   | 7/2007  |
| KR 20040067608 A  | 7/2004  |
| WO 90 02620 A1    | 3/1990  |
| WO 91 10755 A2    | 7/1991  |
| WO 9111540 A1     | 8/1991  |
| WO 9532074 A2     | 11/1995 |
| WO 96/10099 A1    | 4/1996  |
| WO 9833947 A1     | 8/1998  |
| WO 00 37696 A1    | 6/2000  |
| WO 0112868 A1     | 2/2001  |
| WO 02 29139 A2    | 4/2002  |
| WO 03 052154 A1   | 6/2003  |
| WO 03085145 A2    | 10/2003 |
| WO 03085146 A1    | 10/2003 |
| WO 03 104505 A2   | 12/2003 |
| WO 2004 005562 A2 | 1/2004  |
| WO 2004046402 A2  | 6/2004  |
| WO 2005 045080 A1 | 5/2005  |
| WO 2005047554 A1  | 5/2005  |

## OTHER PUBLICATIONS

G.T. Murray and T.A. Lograsso, "Preparation and Characterization of Pure Metals," Properties and Selection: Nonferrous Alloys and Special-Purpose Materials, vol. 2, ASM Handbook, ASM International, 1990, 13 pages total.\*

Cabbibo, M. et al., "A TEM study of the combined effect of severe plastic deformation and (Zr), (Sc+Zr)-containing dispersoids on an Al—Mg—Si alloy" Journal of Materials Science, vol. 41, No. 16, Jun. 6, 2006. pp. 5329-5338.

Litynska-Dobrzynska, L. "Effect of heat treatment on the sequence of phases formation in Al—Mg—Si alloy with Sc and Zr additions." Archives of Metallurgy and Materials. 51 (4), pp. 555-560, 2006.

Litynska-Dobrzynska, L. "Precipitation of Phases in Al—Mg—Si—Cu Alloy with Sc and Zr and Zr Additions During Heat Treatment." Diffusion and Defect Data, Solid State Data, Part B, Solid

(56)

**References Cited**

## OTHER PUBLICATIONS

- Statephenomena. vol. 130, No. Applied Crystallography, Jan. 1, 2007. pp. 163-166.
- Cook, R., et al. "Aluminum and Aluminum Alloy Powders for P/M Applications." The Aluminum Powder Company Limited, Ceracon Inc.
- "Aluminum and Aluminum Alloys." ASM Specialty Handbook. 1993. ASM International. p. 559.
- ASM Handbook, vol. 7 ASM International, Materials Park, OH (1993) p. 396.
- Gangopadhyay, A.K., et al. "Effect of rare-earth atomic radius on the devitrification of Al88RE8Ni4 amorphous alloys." Philosophical Magazine A, 2000, vol. 80, No. 5, pp. 1193-1206.
- Riddle, Y.W., et al. "Improving Recrystallization Resistance in W/Rough Aluminum Alloys with Scandium Addition." Lightweight Alloys for Aerospace Applications VI (pp. 26-39), 2001 TMS Annual Meeting, New Orleans, Louisiana, Feb. 11-15, 2001.
- Baikowski Malakoff Inc. "The many uses of High Purity Alumina." Technical Specs. <http://www.baikowskimalakoff.com/pdf/Rc-Ls.pdf> (2005).
- Lotsko, D.V., et al. "Effect of small additions of transition metals on the structure of Al—Zn—Mg—Zr—Sc alloys." New Level of Properties. Advances in Insect Physiology. Academic Press, vol. 2, Nov. 4, 2002. pp. 535-536.
- Neikov, O.D., et al. "Properties of rapidly solidified powder aluminum alloys for elevated temperatures produced by water atomization." Advances in Powder Metallurgy & Particulate Materials. 2002. pp. 7-14-7-27.
- Harada, Y. et al. "Microstructure of Al3Sc with ternary transition-metal additions." Materials Science and Engineering A329-331 (2002) 686-695.
- Unal, A. et al. "Gas Atomization" from the section "Production of Aluminum and Aluminum-Alloy Powder" ASM Handbook, vol. 7. 2002.
- Riddle, Y.W., et al. "A Study of Coarsening, Recrystallization, and Morphology of Microstructure in Al—Sc—(Zr)—(Mg) Alloys." Metallurgical and Materials Transactions A. vol. 35A, Jan. 2004. pp. 341-350.
- Tian, N. et al. "Heating rate dependence of glass transition and primary crystallization of Al88Gd6Er2Ni4 metallic glass." Scripta Materialia 53 (2005) pp. 681-685.
- Litynska, L. et al. "Experimental and theoretical characterization of Al3Sc precipitates in Al—Mg—Si—Cu—Sc—Zr alloys." Zeitschrift Fur Metallkunde. vol. 97, No. 3. Jan. 1, 2006. pp. 321-324.
- Rachek, O.P. "X-ray diffraction study of amorphous alloys Al—Ni—Ce with using Ehrenfest's formula." Journal of Non-Crystalline Solids 352 (2006) pp. 3781-3786.
- Pandey A B et al, "High Strength Discontinuously Reinforced Aluminum for Rocket Applications," Affordable Metal Matrix Composites for High Performance Applications. Symposia Proceedings, TMS (The Minerals, Metals & Materials Society), US, No. 2nd, Jan. 1, 2008, pp. 3-12.
- Niu, Ben et al. "Influence of addition of 1-15 erbium on microstructure and crystallization behavior of Al—Ni—Y amorphous alloy" Zhongguo Xitu Xuebao, 26(4), pp. 450-454. 2008.
- Riddle, Y.W., et al. "Recrystallization Performance of AA7050 Varied with Sc and Zr." Materials Science Forum. 2000. pp. 799-804.
- Lotsko, D.V., et al. "High-strength aluminum-based alloys hardened by quasicrystalline nanoparticles." Science for Materials in the Frontier of Centuries: Advantages and Challenges, International Conference: Kyiv, Ukraine. Nov. 4-8, 2002. vol. 2. pp. 371-372.
- Hardness Conversion Table. Downloaded from [http://www.gordonengland.co.uk/hardness/hardness\\_conversion\\_2m.htm](http://www.gordonengland.co.uk/hardness/hardness_conversion_2m.htm).

\* cited by examiner

FIG. 1



FIG. 2







FIG. 5







*FIG. 7A*



*FIG. 7B*



*FIG. 8A*



*FIG. 8B*



FIG. 9

## 1

**METHOD FOR PRODUCING HIGH  
STRENGTH ALUMINUM ALLOY POWDER  
CONTAINING L1<sub>2</sub> INTERMETALLIC  
DISPERSOIDS**

**CROSS-REFERENCE TO RELATED  
APPLICATION(S)**

This application is related to the following co-pending applications that are filed on even date herewith and are assigned to the same assignee: VERSION PROCESS FOR HEAT TREATABLE L1<sub>2</sub> ALUMINUM ALLOYS, Ser. No. 12/316,020; and A METHOD FOR FORMING HIGH STRENGTH ALUMINUM ALLOYS CONTAINING L1<sub>2</sub> INTERMETALLIC DISPERSOIDS, Ser. No. 12/316,046.

This application is also related to the following co-pending applications that were filed on Apr. 18, 2008, and are assigned to the same assignee: L1<sub>2</sub> ALUMINUM ALLOYS WITH BIMODAL AND TRIMODAL DISTRIBUTION, Ser. No. 12/148,395; DISPERSION STRENGTHENED L1<sub>2</sub> ALUMINUM ALLOYS, Ser. No. 12/148,432; HEAT TREATABLE L1<sub>2</sub> ALUMINUM ALLOYS, Ser. No. 12/148,383; HIGH STRENGTH L1<sub>2</sub> ALUMINUM ALLOYS, Ser. No. 12/148,394; HIGH STRENGTH L1<sub>2</sub> ALUMINUM ALLOYS, Ser. No. 12/148,382; HEAT TREATABLE L1<sub>2</sub> ALUMINUM ALLOYS, Ser. No. 12/148,396; HIGH STRENGTH L1<sub>2</sub> ALUMINUM ALLOYS, Ser. No. 12/148,387; HIGH STRENGTH ALUMINUM ALLOYS WITH L1<sub>2</sub> PRECIPITATES, Ser. No. 12/148,426; HIGH STRENGTH L1<sub>2</sub> ALUMINUM ALLOYS, Ser. No. 12/148,459; and L1<sub>2</sub> STRENGTHENED AMORPHOUS ALUMINUM ALLOYS, Ser. No. 12/148,458.

**BACKGROUND**

The present invention relates generally to aluminum alloys and more specifically to a method for forming high strength aluminum alloy powder having L1<sub>2</sub> dispersoids therein.

The combination of high strength, ductility, and fracture toughness, as well as low density, make aluminum alloys natural candidates for aerospace and space applications. However, their use is typically limited to temperatures below about 300° F. (149° C.) since most aluminum alloys start to lose strength in that temperature range as a result of coarsening of strengthening precipitates.

The development of aluminum alloys with improved elevated temperature mechanical properties is a continuing process. Some attempts have included aluminum-iron and aluminum-chromium based alloys such as Al—Fe—Ce, Al—Fe—V—Si, Al—Fe—Ce—W, and Al—Cr—Zr—Mn that contain incoherent dispersoids. These alloys, however, also lose strength at elevated temperatures due to particle coarsening. In addition, these alloys exhibit ductility and fracture toughness values lower than other commercially available aluminum alloys.

Other attempts have included the development of mechanically alloyed Al—Mg and Al—Ti alloys containing ceramic dispersoids. These alloys exhibit improved high temperature strength due to the particle dispersion, but the ductility and fracture toughness are not improved.

U.S. Pat. No. 6,248,453 owned by the assignee of the present application discloses aluminum alloys strengthened by dispersed Al<sub>3</sub>X L1<sub>2</sub> intermetallic phases where X is selected from the group consisting of Sc, Er, Lu, Yb, Tm, and Lu. The Al<sub>3</sub>X particles are coherent with the aluminum alloy matrix and are resistant to coarsening at elevated temperatures. The improved mechanical properties of the disclosed

## 2

dispersion strengthened L1<sub>2</sub> aluminum alloys are stable up to 572° F. (300° C.). U.S. Patent Application Publication No. 2006/0269437 Al, also commonly owned, discloses a high strength aluminum alloy that contains scandium and other elements that is strengthened by L1<sub>2</sub> dispersoids.

L1<sub>2</sub> strengthened aluminum alloys have high strength and improved fatigue properties compared to commercially available aluminum alloys. Fine grain size results in improved mechanical properties of materials. Hall-Petch strengthening has been known for decades where strength increases as grain size decreases. An optimum grain size for optimum strength is in the nano range of about 30 to 100 nm. These alloys also have lower ductility.

**SUMMARY**

The present invention is a method for forming aluminum alloy powders that can be processed into alloys with high temperature strength and acceptable fracture toughness. In embodiments, powders include an aluminum alloy having coherent L1<sub>2</sub> Al<sub>3</sub>X dispersoids where X is at least one first element selected from scandium, erbium, thulium, ytterbium, and lutetium, and at least one second element selected from gadolinium, yttrium, zirconium, titanium, hafnium, and niobium. The balance is substantially aluminum containing at least one alloying element selected from silicon, magnesium, lithium, copper, zinc, and nickel.

The powders are formed by high pressure gas atomization of molten aluminum alloys containing L1<sub>2</sub> dispersoid forming elements. The melted alloy is contacted with a high velocity inert gas stream to form liquid droplets followed by rapid cooling. Control of the gas pressure and melt flow rate controls the size of the droplets and, after solidification, the size of the powder. The alloy melt is heated to a superheat temperature of from about 150° F. (66° C.) to about 200° F. (93° C.) above the melting point of the melt.

The inert gas is preferably selected from nitrogen, argon and helium. The oxygen content of the resulting powder is between about 1 ppm and 2000 ppm, preferred about 10 ppm to 1000 ppm and most preferred about 25 ppm to about 500 ppm and the hydrogen content is about 1 ppm to about 1000 ppm, preferred about 5 ppm to 500 ppm and most preferred about 25 ppm to about 200 ppm.

The mean powder size is between about 1 micron to about 250 microns preferred about 5 microns to about 100 microns and most preferred about 5 microns to about 50 microns.

**BRIEF DESCRIPTION OF THE DRAWINGS**

- FIG. 1 is an aluminum scandium phase diagram.
- FIG. 2 is an aluminum erbium phase diagram.
- FIG. 3 is an aluminum thulium phase diagram.
- FIG. 4 is an aluminum ytterbium phase diagram.
- FIG. 5 is an aluminum lutetium phase diagram.
- FIG. 6A is a schematic diagram of a vertical gas atomizer.
- FIG. 6B is a close up view of nozzle 108 in FIG. 6A.
- FIGS. 7A and 7B are SEM photos of the inventive aluminum alloy powder.
- FIGS. 8A and 8B are optical micrographs showing the microstructure of gas atomized L1<sub>2</sub> aluminum alloy powder.
- FIG. 9 is a diagram of the gas atomization process.

**DETAILED DESCRIPTION**

**1. L1<sub>2</sub> Alloys**

The alloy powders of this invention are formed from aluminum based alloys with high strength and fracture tough-

ness for applications at temperatures from about  $-420^{\circ}$  F. ( $-251^{\circ}$  C.) up to about  $650^{\circ}$  F. ( $343^{\circ}$  C.). The aluminum alloys comprise a solid solution of aluminum and at least one element selected from silicon, magnesium, lithium, copper, zinc, and nickel strengthened by  $L1_2$   $Al_3X$  coherent precipitates where X is at least one first element selected from scandium, erbium, thulium, ytterbium, and lutetium, and at least one second element selected from gadolinium, yttrium, zirconium, titanium, hafnium, and niobium.

The aluminum silicon system is a simple eutectic alloy system with a eutectic reaction at 12.5 weight percent silicon and  $1077^{\circ}$  F. ( $577^{\circ}$  C.). There is little solubility of silicon in aluminum at temperatures up to  $930^{\circ}$  F. ( $500^{\circ}$  C.) and none of aluminum in silicon. However, the solubility can be extended significantly by utilizing rapid solidification techniques.

The binary aluminum magnesium system is a simple eutectic at 36 weight percent magnesium and  $842^{\circ}$  F. ( $450^{\circ}$  C.). There is complete solubility of magnesium and aluminum in the rapidly solidified aluminum alloys discussed herein.

The binary aluminum lithium system is a simple eutectic at 8 weight percent lithium and  $1105^{\circ}$  F. ( $596^{\circ}$  C.). The equilibrium solubility of 4 weight percent lithium can be extended significantly by rapid solidification techniques. There can be complete solubility of lithium in the rapidly solidified aluminum alloys discussed herein.

The binary aluminum copper system is a simple eutectic at 32 weight percent copper and  $1018^{\circ}$  F. ( $548^{\circ}$  C.). There can be complete solubility of copper in the rapidly solidified aluminum alloys discussed herein.

The aluminum zinc binary system is a eutectic alloy system involving a monotectoid reaction and a miscibility gap in the solid state. There is a eutectic reaction at 94 weight percent zinc and  $718^{\circ}$  F. ( $381^{\circ}$  C.). Zinc has maximum solid solubility of 83.1 weight percent in aluminum at  $717.8^{\circ}$  F. ( $381^{\circ}$  C.) which can be extended by rapid solidification processes. Decomposition of the supersaturated solid solution of zinc in aluminum gives rise to spherical and ellipsoidal Guinier Preston (GP) zones which are aluminum and zinc rich clusters that are coherent with the matrix and act to strengthen the alloy.

The aluminum nickel binary system is a simple eutectic at 5.7 weight percent nickel and  $1183.8^{\circ}$  F. ( $639.9^{\circ}$  C.). There is little solubility of nickel in aluminum. However, the solubility can be extended significantly by utilizing rapid solidification processes. The equilibrium phase in the aluminum nickel eutectic system is  $L1_2$  intermetallic  $Al_3Ni$ .

In the aluminum based alloys disclosed herein, scandium, erbium, thulium, ytterbium, and lutetium are potent strengtheners that have low diffusivity and low solubility in aluminum. All these elements form equilibrium  $Al_3X$  intermetallic dispersoids where X is at least one of scandium, erbium, thulium, ytterbium, and lutetium, that have an  $L1_2$  structure that is an ordered face centered cubic structure with the X atoms located at the corners and aluminum atoms located on the cube faces of the unit cell.

Scandium forms  $Al_3Sc$  dispersoids that are fine and coherent with the aluminum matrix. Lattice parameters of aluminum and  $Al_3Sc$  are very close (0.405 nm and 0.410 nm respectively), indicating that there is minimal or no driving force for causing growth of the  $Al_3Sc$  dispersoids. This low interfacial energy makes the  $Al_3Sc$  dispersoids thermally stable and resistant to coarsening up to temperatures as high as about  $842^{\circ}$  F. ( $450^{\circ}$  C.). Additions of magnesium in aluminum increase the lattice parameter of the aluminum matrix, and decrease the lattice parameter mismatch, further increasing the resistance of the  $Al_3Sc$  to coarsening. Additions of zinc, copper, lithium, silicon, and nickel provide solid solution and

precipitation strengthening in the aluminum alloys. These  $Al_3Sc$  dispersoids are made stronger and more resistant to coarsening at elevated temperatures by adding suitable alloying elements such as gadolinium, yttrium, zirconium, titanium, hafnium, niobium, or combinations thereof, that enter  $Al_3Sc$  in solution.

Erbium forms  $Al_3Er$  dispersoids in the aluminum matrix that are fine and coherent with the aluminum matrix. The lattice parameters of aluminum and  $Al_3Er$  are close (0.405 nm and 0.417 nm respectively), indicating there is minimal driving force for causing growth of the  $Al_3Er$  dispersoids. This low interfacial energy makes the  $Al_3Er$  dispersoids thermally stable and resistant to coarsening up to temperatures as high as about  $842^{\circ}$  F. ( $450^{\circ}$  C.). Additions of magnesium in aluminum increase the lattice parameter of the aluminum matrix, and decrease the lattice parameter mismatch, further increasing the resistance of the  $Al_3Er$  to coarsening. Additions of zinc, copper, lithium, silicon, and nickel provide solid solution and precipitation strengthening in the aluminum alloys.

These  $Al_3Er$  dispersoids are made stronger and more resistant to coarsening at elevated temperatures by adding suitable alloying elements such as gadolinium, yttrium, zirconium, titanium, hafnium, niobium, or combinations thereof that enter  $Al_3Er$  in solution.

Thulium forms metastable  $Al_3Tm$  dispersoids in the aluminum matrix that are fine and coherent with the aluminum matrix. The lattice parameters of aluminum and  $Al_3Tm$  are close (0.405 nm and 0.420 nm respectively), indicating there is minimal driving force for causing growth of the  $Al_3Tm$  dispersoids. This low interfacial energy makes the  $Al_3Tm$  dispersoids thermally stable and resistant to coarsening up to temperatures as high as about  $842^{\circ}$  F. ( $450^{\circ}$  C.). Additions of magnesium in aluminum increase the lattice parameter of the aluminum matrix, and decrease the lattice parameter mismatch, further increasing the resistance of the  $Al_3Tm$  to coarsening. Additions of zinc, copper, lithium, silicon, and nickel provide solid solution and precipitation strengthening in the aluminum alloys. These  $Al_3Tm$  dispersoids are made stronger and more resistant to coarsening at elevated temperatures by adding suitable alloying elements such as gadolinium, yttrium, zirconium, titanium, hafnium, niobium, or combinations thereof that enter  $Al_3Tm$  in solution.

Ytterbium forms  $Al_3Yb$  dispersoids in the aluminum matrix that are fine and coherent with the aluminum matrix.

45 The lattice parameters of Al and  $Al_3Yb$  are close (0.405 nm and 0.420 nm respectively), indicating there is minimal driving force for causing growth of the  $Al_3Yb$  dispersoids. This low interfacial energy makes the  $Al_3Yb$  dispersoids thermally stable and resistant to coarsening up to temperatures as high as about  $842^{\circ}$  F. ( $450^{\circ}$  C.). Additions of magnesium in aluminum increase the lattice parameter of the aluminum matrix, and decrease the lattice parameter mismatch, further increasing the resistance of the  $Al_3Yb$  to coarsening. Additions of zinc, copper, lithium, silicon, and nickel provide solid solution and precipitation strengthening in the aluminum alloys.

55 These  $Al_3Yb$  dispersoids are made stronger and more resistant to coarsening at elevated temperatures by adding suitable alloying elements such as gadolinium, yttrium, zirconium, titanium, hafnium, niobium, or combinations thereof that enter  $Al_3Yb$  in solution.

Lutetium forms  $Al_3Lu$  dispersoids in the aluminum matrix that are fine and coherent with the aluminum matrix. The lattice parameters of Al and  $Al_3Lu$  are close (0.405 nm and 0.419 nm respectively), indicating there is minimal driving force for causing growth of the  $Al_3Lu$  dispersoids. This low interfacial energy makes the  $Al_3Lu$  dispersoids thermally stable and resistant to coarsening up to temperatures as high

## 5

as about 842° F. (450° C.). Additions of magnesium in aluminum increase the lattice parameter of the aluminum matrix, and decrease the lattice parameter mismatch, further increasing the resistance of the  $\text{Al}_3\text{Lu}$  to coarsening. Additions of zinc, copper, lithium, silicon, and nickel provide solid solution and precipitation strengthening in the aluminum alloys. These  $\text{Al}_3\text{Lu}$  dispersoids are made stronger and more resistant to coarsening at elevated temperatures by adding suitable alloying elements such as gadolinium, yttrium, zirconium, titanium, hafnium, niobium, or mixtures thereof that enter  $\text{Al}_3\text{Lu}$  in solution.

Gadolinium forms metastable  $\text{Al}_3\text{Gd}$  dispersoids in the aluminum matrix that are stable up to temperatures as high as about 842° F. (450° C.) due to their low diffusivity in aluminum. The  $\text{Al}_3\text{Gd}$  dispersoids have a  $\text{D}0_{19}$  structure in the equilibrium condition. Despite its large atomic size, gadolinium has fairly high solubility in the  $\text{Al}_3\text{X}$  intermetallic dispersoids (where X is scandium, erbium, thulium, ytterbium or lutetium). Gadolinium can substitute for the X atoms in  $\text{Al}_3\text{X}$  intermetallic, thereby forming an ordered  $\text{L}1_2$  phase, which results in improved thermal and structural stability.

Yttrium forms metastable  $\text{Al}_3\text{Y}$  dispersoids in the aluminum matrix that have an  $\text{L}1_2$  structure in the metastable condition and a  $\text{D}0_{19}$  structure in the equilibrium condition. The metastable  $\text{Al}_3\text{Y}$  dispersoids have a low diffusion coefficient which makes them thermally stable and highly resistant to coarsening. Yttrium has a high solubility in the  $\text{Al}_3\text{X}$  intermetallic dispersoids allowing large amounts of yttrium to substitute for X in the  $\text{Al}_3\text{X}$   $\text{L}1_2$  dispersoids, which results in improved thermal and structural stability.

Zirconium forms  $\text{Al}_3\text{Zr}$  dispersoids in the aluminum matrix that have an  $\text{L}1_2$  structure in the metastable condition and  $\text{D}0_{23}$  structure in the equilibrium condition. The metastable  $\text{Al}_3\text{Zr}$  dispersoids have a low diffusion coefficient which makes them thermally stable and highly resistant to coarsening. Zirconium has a high solubility in the  $\text{Al}_3\text{X}$  dispersoids allowing large amounts of zirconium to substitute for X in the  $\text{Al}_3\text{X}$  dispersoids, which results in improved thermal and structural stability.

Titanium forms  $\text{Al}_3\text{Ti}$  dispersoids in the aluminum matrix that have an  $\text{L}1_2$  structure in the metastable condition and  $\text{D}0_{22}$  structure in the equilibrium condition. The metastable  $\text{Al}_3\text{Ti}$  dispersoids have a low diffusion coefficient which makes them thermally stable and highly resistant to coarsening. Titanium has a high solubility in the  $\text{Al}_3\text{X}$  dispersoids allowing large amounts of titanium to substitute for X in the  $\text{Al}_3\text{X}$  dispersoids, which results in improved thermal and structural stability.

Hafnium forms metastable  $\text{Al}_3\text{Hf}$  dispersoids in the aluminum matrix that have an  $\text{L}1_2$  structure in the metastable condition and a  $\text{D}0_{23}$  structure in the equilibrium condition. The  $\text{Al}_3\text{Hf}$  dispersoids have a low diffusion coefficient, which makes them thermally stable and highly resistant to coarsening. Hafnium has a high solubility in the  $\text{Al}_3\text{X}$  dispersoids allowing large amounts of hafnium to substitute for scandium, erbium, thulium, ytterbium, and lutetium in the above mentioned  $\text{Al}_3\text{X}$  dispersoids, which results in stronger and more thermally stable dispersoids.

Niobium forms metastable  $\text{Al}_3\text{Nb}$  dispersoids in the aluminum matrix that have an  $\text{L}1_2$  structure in the metastable condition and a  $\text{D}0_{22}$  structure in the equilibrium condition. Niobium has a lower solubility in the  $\text{Al}_3\text{X}$  dispersoids than hafnium or yttrium, allowing relatively lower amounts of niobium than hafnium or yttrium to substitute for X in the  $\text{Al}_3\text{X}$  dispersoids. Nonetheless, niobium can be very effective in slowing down the coarsening kinetics of the  $\text{Al}_3\text{X}$  dispersoids because the  $\text{Al}_3\text{Nb}$  dispersoids are thermally stable. The

## 6

substitution of niobium for X in the above mentioned  $\text{Al}_3\text{X}$  dispersoids results in stronger and more thermally stable dispersoids.

$\text{Al}_3\text{X}$   $\text{L}1_2$  precipitates improve elevated temperature mechanical properties in aluminum alloys for two reasons. First, the precipitates are ordered intermetallic compounds. As a result, when the particles are sheared by glide dislocations during deformation, the dislocations separate into two partial dislocations separated by an anti-phase boundary on the glide plane. The energy to create the anti-phase boundary is the origin of the strengthening. Second, the cubic  $\text{L}1_2$  crystal structure and lattice parameter of the precipitates are closely matched to the aluminum solid solution matrix. This results in a lattice coherency at the precipitate/matrix boundary that resists coarsening. The lack of an interphase boundary results in a low driving force for particle growth and resulting elevated temperature stability. Alloying elements in solid solution in the dispersed strengthening particles and in the aluminum matrix that tend to decrease the lattice mismatch between the matrix and particles will tend to increase the strengthening and elevated temperature stability of the alloy.

$\text{L}1_2$  phase strengthened aluminum alloys are important structural materials because of their excellent mechanical properties and the stability of these properties at elevated temperature due to the resistance of the coherent dispersoids in the microstructure to particle coarsening. The mechanical properties are optimized by maintaining a high volume fraction of  $\text{L}1_2$  dispersoids in the microstructure. The  $\text{L}1_2$  dispersoid concentration following aging scales as the amount of  $\text{L}1_2$  phase forming elements in solid solution in the aluminum alloy following quenching. Examples of  $\text{L}1_2$  phase forming elements include but are not limited to Sc, Er, Th, Yb, and Lu. The concentration of alloying elements in solid solution in alloys cooled from the melt is directly proportional to the cooling rate.

Exemplary aluminum alloys for the bimodal system alloys of this invention include, but are not limited to (in weight percent unless otherwise specified):

- 40 about  $\text{Al}-\text{M}-(0.1-4)\text{Sc}-(0.1-20)\text{Gd};$
- about  $\text{Al}-\text{M}-(0.1-20)\text{Er}-(0.1-20)\text{Gd};$
- about  $\text{Al}-\text{M}-(0.1-15)\text{Tm}-(0.1-20)\text{Gd};$
- about  $\text{Al}-\text{M}-(0.1-25)\text{Yb}-(0.1-20)\text{Gd};$
- about  $\text{Al}-\text{M}-(0.1-25)\text{Lu}-(0.1-20)\text{Gd};$
- about  $\text{Al}-\text{M}-(0.1-4)\text{Sc}-(0.1-20)\text{Y};$
- about  $\text{Al}-\text{M}-(0.1-20)\text{Er}-(0.1-20)\text{Y};$
- about  $\text{Al}-\text{M}-(0.1-15)\text{Tm}-(0.1-20)\text{Y};$
- 30 about  $\text{Al}-\text{M}-(0.1-25)\text{Yb}-(0.1-20)\text{Y};$
- about  $\text{Al}-\text{M}-(0.1-25)\text{Lu}-(0.1-20)\text{Y};$
- about  $\text{Al}-\text{M}-(0.1-4)\text{Sc}-(0.05-4)\text{Zr};$
- about  $\text{Al}-\text{M}-(0.1-20)\text{Er}-(0.05-4)\text{Zr};$
- about  $\text{Al}-\text{M}-(0.1-15)\text{Tm}-(0.05-4)\text{Zr};$
- 45 about  $\text{Al}-\text{M}-(0.1-25)\text{Yb}-(0.05-4)\text{Zr};$
- about  $\text{Al}-\text{M}-(0.1-25)\text{Lu}-(0.05-4)\text{Zr};$
- about  $\text{Al}-\text{M}-(0.1-4)\text{Sc}-(0.05-10)\text{Ti};$
- about  $\text{Al}-\text{M}-(0.1-20)\text{Er}-(0.05-10)\text{Ti};$
- about  $\text{Al}-\text{M}-(0.1-15)\text{Tm}-(0.05-10)\text{Ti};$
- 55 about  $\text{Al}-\text{M}-(0.1-25)\text{Yb}-(0.05-10)\text{Ti};$
- about  $\text{Al}-\text{M}-(0.1-25)\text{Lu}-(0.05-10)\text{Ti};$
- about  $\text{Al}-\text{M}-(0.1-4)\text{Sc}-(0.05-10)\text{Hf};$
- about  $\text{Al}-\text{M}-(0.1-20)\text{Er}-(0.05-10)\text{Hf};$
- about  $\text{Al}-\text{M}-(0.1-15)\text{Tm}-(0.05-10)\text{Hf};$
- 60 about  $\text{Al}-\text{M}-(0.1-25)\text{Yb}-(0.05-10)\text{Hf};$
- about  $\text{Al}-\text{M}-(0.1-25)\text{Lu}-(0.05-10)\text{Hf};$
- about  $\text{Al}-\text{M}-(0.1-4)\text{Sc}-(0.05-5)\text{Nb};$
- about  $\text{Al}-\text{M}-(0.1-20)\text{Er}-(0.05-5)\text{Nb};$
- 65 about  $\text{Al}-\text{M}-(0.1-15)\text{Tm}-(0.05-5)\text{Nb};$

about Al-M-(0.1-25)Yb-(0.05-5)Nb; and about Al-M-(0.1-25)Lu-(0.05-5)Nb.

M is at least one of about (4-25) weight percent silicon, (1-8) weight percent magnesium, (0.5-3) weight percent lithium, (0.2-3) weight percent copper, (3-12) weight percent zinc, and (1-12) weight percent nickel.

The amount of silicon present in the fine grain matrix, if any, may vary from about 4 to about 25 weight percent, more preferably from about 4 to about 18 weight percent, and even more preferably from about 5 to about 11 weight percent.

The amount of magnesium present in the fine grain matrix, if any, may vary from about 1 to about 8 weight percent, more preferably from about 3 to about 7.5 weight percent, and even more preferably from about 4 to about 6.5 weight percent.

The amount of lithium present in the fine grain matrix, if any, may vary from about 0.5 to about 3 weight percent, more preferably from about 1 to about 2.5 weight percent, and even more preferably from about 1 to about 2 weight percent.

The amount of copper present in the fine grain matrix, if any, may vary from about 0.2 to about 6 weight percent, more preferably from about 0.5 to about 5 weight percent, and even more preferably from about 2 to about 5.0 weight percent.

The amount of zinc present in the fine grain matrix, if any, may vary from about 3 to about 12 weight percent, more preferably from about 4 to about 10 weight percent, and even more preferably from about 5 to about 9 weight percent.

The amount of nickel present in the fine grain matrix, if any, vary from about 1 to about 12 weight percent, more preferably from about 2 to about 10 weight percent, and even more preferably from about 4 to about 10 weight percent.

The amount of scandium present in the fine grain matrix, if any, may vary from 0.1 to about 4 weight percent, more preferably from about 0.1 to about 3 weight percent, and even more preferably from about 0.2 to about 2.5 weight percent. The Al—Sc phase diagram shown in FIG. 1 indicates a eutectic reaction at about 0.5 weight percent scandium at about 1219° F. (659° C.) resulting in a solid solution of scandium and aluminum and Al<sub>3</sub>Sc dispersoids. Aluminum alloys with less than 0.5 weight percent scandium can be quenched from the melt to retain scandium in solid solution that may precipitate as dispersed L1<sub>2</sub> intermetallic Al<sub>3</sub>Sc following an aging treatment. Alloys with scandium in excess of the eutectic composition (hypereutectic alloys) can only retain scandium in solid solution by rapid solidification processing (RSP) where cooling rates are in excess of about 10<sup>3</sup>° C./second.

The amount of erbium present in the fine grain matrix, if any, may vary from about 0.1 to about 20 weight percent, more preferably from about 0.3 to about 15 weight percent, and even more preferably from about 0.5 to about 10 weight percent. The Al—Er phase diagram shown in FIG. 2 indicates a eutectic reaction at about 6 weight percent erbium at about 1211° F. (655° C.). Aluminum alloys with less than about 6 weight percent erbium can be quenched from the melt to retain erbium in solid solutions that may precipitate as dispersed L1<sub>2</sub> intermetallic Al<sub>3</sub>Er following an aging treatment. Alloys with erbium in excess of the eutectic composition can only retain erbium in solid solution by rapid solidification processing (RSP) where cooling rates are in excess of about 10<sup>3</sup>° C./second.

The amount of thulium present in the alloys, if any, may vary from about 0.1 to about 15 weight percent, more preferably from about 0.2 to about 10 weight percent, and even more preferably from about 0.4 to about 6 weight percent. The Al—Tm phase diagram shown in FIG. 3 indicates a eutectic reaction at about 10 weight percent thulium at about 1193° F. (645° C.). Thulium forms metastable Al<sub>3</sub>Tm dispersoids in the aluminum matrix that have an L1<sub>2</sub> structure in the

equilibrium condition. The Al<sub>3</sub>Tm dispersoids have a low diffusion coefficient which makes them thermally stable and highly resistant to coarsening. Aluminum alloys with less than 10 weight percent thulium can be quenched from the melt to retain thulium in solid solution that may precipitate as dispersed metastable L1<sub>2</sub> intermetallic Al<sub>3</sub>Tm following an aging treatment. Alloys with thulium in excess of the eutectic composition can only retain Tm in solid solution by rapid solidification processing (RSP) where cooling rates are in excess of about 10<sup>3</sup>° C./second.

The amount of ytterbium present in the alloys, if any, may vary from about 0.1 to about 25 weight percent, more preferably from about 0.3 to about 20 weight percent, and even more preferably from about 0.4 to about 10 weight percent.

The Al—Yb phase diagram shown in FIG. 4 indicates a eutectic reaction at about 21 weight percent ytterbium at about 1157° F. (625° C.). Aluminum alloys with less than about 21 weight percent ytterbium can be quenched from the melt to retain ytterbium in solid solution that may precipitate as dispersed L1<sub>2</sub> intermetallic Al<sub>3</sub>Yb following an aging treatment. Alloys with ytterbium in excess of the eutectic composition can only retain ytterbium in solid solution by rapid solidification processing (RSP) where cooling rates are in excess of about 10<sup>3</sup>° C. per second.

The amount of lutetium present in the alloys, if any, may vary from about 0.1 to about 25 weight percent, more preferably from about 0.3 to about 20 weight percent, and even more preferably from about 0.4 to about 10 weight percent.

The Al—Lu phase diagram shown in FIG. 5 indicates a eutectic reaction at about 11.7 weight percent Lu at about 1202° F. (650° C.). Aluminum alloys with less than about 11.7 weight percent lutetium can be quenched from the melt to retain Lu in solid solution that may precipitate as dispersed L1<sub>2</sub> intermetallic Al<sub>3</sub>Lu following an aging treatment. Alloys with Lu in excess of the eutectic composition can only retain Lu in solid solution by rapid solidification processing (RSP) where cooling rates are in excess of about 10<sup>3</sup>° C./second.

The amount of gadolinium present in the alloys, if any, may vary from about 0.1 to about 20 weight percent, more preferably from about 0.3 to about 15 weight percent, and even more preferably from about 0.5 to about 10 weight percent.

The amount of yttrium present in the alloys, if any, may vary from about 0.1 to about 20 weight percent, more preferably from about 0.3 to about 15 weight percent, and even more preferably from about 0.5 to about 10 weight percent.

The amount of zirconium present in the alloys, if any, may vary from about 0.05 to about 4 weight percent, more preferably from about 0.1 to about 3 weight percent, and even more preferably from about 0.3 to about 2 weight percent.

The amount of titanium present in the alloys, if any, may vary from about 0.05 to about 10 weight percent, more preferably from about 0.2 to about 8 weight percent, and even more preferably from about 0.4 to about 4 weight percent.

The amount of hafnium present in the alloys, if any, may vary from about 0.05 to about 10 weight percent, more preferably from about 0.2 to about 8 weight percent, and even more preferably from about 0.4 to about 5 weight percent.

The amount of niobium present in the alloys, if any, may vary from about 0.05 to about 5 weight percent, more preferably from about 0.1 to about 3 weight percent, and even more preferably from about 0.2 to about 2 weight percent.

In order to have the best properties for the fine grain matrix, it is desirable to limit the amount of other elements. Specific elements that should be reduced or eliminated include no more than about 0.1 weight percent iron, 0.1 weight percent chromium, 0.1 weight percent manganese, 0.1 weight percent vanadium, and 0.1 weight percent cobalt. The total quantity of

additional elements should not exceed about 1% by weight, including the above listed impurities and other elements.

## 2. L1<sub>2</sub> Alloy Powder Formation

The highest cooling rates observed in commercially viable processes are achieved by gas atomization of molten metals to produce powder. Gas atomization is a two fluid process wherein a stream of molten metal is disintegrated by a high velocity gas stream. The end result is that the particles of molten metal eventually become spherical due to surface tension and finely solidify in powder form. Heat from the liquid droplets is transferred to the atomization gas by convection. The solidification rates, depending on the gas and the surrounding environment, can be very high and can exceed 10<sup>60</sup> C./second. Cooling rates greater than 10<sup>30</sup> C./second are typically specified to ensure supersaturation of alloying elements in gas atomized L1<sub>2</sub> aluminum alloy powder in the inventive process described herein.

A schematic of typical vertical gas atomizer 100 is shown in FIG. 6A. FIG. 6A is taken from R. Germain, Powder Metallurgy Science Second Edition MPIF (1994) (chapter 3, p. 101) and is included herein for reference. Vacuum or inert gas induction melter 102 is positioned at the top of free flight chamber 104. Vacuum induction melter 102 contains melt 106 which flows by gravity or gas overpressure through nozzle 108. A close up view of nozzle 108 is shown in FIG. 6B. Melt 106 enters nozzle 108 and flows downward till it meets high pressure gas stream from gas source 110 where it is transformed into a spray of droplets. The droplets eventually become spherical due to surface tension and rapidly solidify into spherical powder 112 which collects in collection chamber 114. The gas recirculates through cyclone collector 116 which collects fine powder 118 before returning to the input gas stream. As can be seen from FIG. 6A, the surroundings to which the melt and eventual powder are exposed are completely controlled.

There are many effective nozzle designs known in the art to produce spherical metal powder. Designs with short gas-to-melt separation distances produce finer powders. Confined nozzle designs where gas meets the molten stream at a short distance just after it leaves the atomization nozzle are preferred for the production of the inventive L1<sub>2</sub> aluminum alloy powders disclosed herein. Higher superheat temperatures cause lower melt viscosity and longer cooling times. Both result in smaller spherical particles.

A large number of processing parameters are associated with gas atomization that affect the final product. Examples include melt superheat, gas pressure, metal flow rate, gas type, and gas purity. In gas atomization, the particle size is related to the energy input to the metal. Higher gas pressures, higher superheat temperatures and lower metal flow rates result in smaller particle sizes. Higher gas pressures provide higher gas velocities for a given atomization nozzle design.

To maintain purity, inert gases are used, such as helium, argon, and nitrogen. Helium is preferred for rapid solidification because the high heat transfer coefficient of the gas leads to high quenching rates and high supersaturation of alloying elements.

Lower metal flow rates and higher gas flow ratios favor production of finer powders. The particle size of gas atomized melts typically has a log normal distribution. In the turbulent conditions existing at the gas/metal interface during atomization, ultra fine particles can form that may reenter the gas expansion zone. These solidified fine particles can be carried into the flight path of molten larger droplets resulting in agglomeration of small satellite particles on the surfaces of

larger particles. An example of small satellite particles attached to inventive spherical L1<sub>2</sub> aluminum alloy powder is shown in the scanning electron microscopy (SEM) micrographs of FIGS. 7A and 7B at two magnifications. The spherical shape of gas atomized aluminum powder is evident. The spherical shape of the powder is suggestive of clean powder without excessive oxidation. Higher oxygen in the powder results in irregular powder shape. Spherical powder helps in improving the flowability of powder which results in higher apparent density and tap density of the powder. The satellite particles can be minimized by adjusting processing parameters to reduce or even eliminate turbulence in the gas atomization process. The microstructure of gas atomized aluminum alloy powder is predominantly cellular as shown in the optical micrographs of cross-sections of the inventive alloy in FIGS. 8A and 8B at two magnifications. The rapid cooling rate suppresses dendritic solidification common at slower cooling rates resulting in a finer microstructure with minimum alloy segregation.

Oxygen and hydrogen in the powder can degrade the mechanical properties of the final part. It is preferred to limit the oxygen in the L1<sub>2</sub> alloy powder to about 1 ppm to 2000 ppm. Oxygen is intentionally introduced as a component of the helium gas during atomization. An oxide coating on the L1<sub>2</sub> aluminum powder is beneficial for two reasons. First, the coating prevents agglomeration by contact sintering and secondly, the coating inhibits the chance of explosion of the powder. A controlled amount of oxygen is important in order to provide good ductility and fracture toughness in the final consolidated material. Hydrogen content in the powder is controlled by ensuring the dew point of the helium gas is low. A dew point of about minus 50° F. (minus 45.5° C.) to minus 100° F. (minus 73.3° C.) is preferred.

In preparation for final processing, the powder is classified according to size by sieving. To prepare the powder for sieving, if the powder has zero percent oxygen content, the powder may be exposed to nitrogen gas which passivates the powder surface and prevents agglomeration. Finer powder sizes result in improved mechanical properties of the end product. While minus 325 mesh (about 45 microns) powder can be used, minus 450 mesh (about 30 microns) powder is a preferred size in order to provide good mechanical properties in the end product. During the atomization process, powder is collected in collection chambers in order to prevent oxidation of the powder. Collection chambers are used at the bottom of atomization chamber 104 as well as at the bottom of cyclone collector 116. The powder is transported and stored in the collection chambers also. Collection chambers are maintained under positive pressure with nitrogen gas which prevents oxidation of the powder.

A schematic of the L1<sub>2</sub> aluminum powder manufacturing process is shown in FIG. 9. In the process aluminum 200 and L1<sub>2</sub> forming (and other alloying elements) 210 are melted in furnace 220 to a predetermined superheat temperature under vacuum or inert atmosphere. Preferred charge for furnace 220 is prealloyed aluminum 200 and L1<sub>2</sub> and other alloying elements before charging furnace 220. Melt 230 is then passed through nozzle 240 where it is impacted by pressurized gas stream 250. Gas stream 250 is an inert gas such as nitrogen, argon or helium, preferably helium. Melt 230 can flow through nozzle 240 under gravity or under pressure. Gravity flow is preferred for the inventive process disclosed herein. Preferred pressures for pressurized gas stream 250 are about 50 psi (10.35 MPa) to about 750 psi (5.17 MPa) depending on the alloy.

The atomization process creates molten droplets 260 which rapidly solidify as they travel through chamber 270

forming spherical powder particles 280. The molten droplets transfer heat to the atomizing gas by convection. The role of the atomizing gas is two fold: one is to disintegrate the molten metal stream into fine droplets by transferring kinetic energy from the gas to the melt stream and the other is to extract heat from the molten droplets to rapidly solidify them into spherical powder. The solidification time and cooling rate vary with droplet size. Larger droplets take longer to solidify and their resulting cooling rate is lower. On the other hand, the atomizing gas will extract heat efficiently from smaller droplets resulting in a higher cooling rate. Finer powder size is therefore preferred as higher cooling rates provide finer microstructures and higher mechanical properties in the end product. Higher cooling rates lead to finer cellular microstructures which are preferred for higher mechanical properties. Finer cellular microstructures result in finer grain sizes in consolidated product. Finer grain size provides higher yield strength of the material through the Hall-Petch strengthening model.

Key process variables for gas atomization include superheat temperature, nozzle diameter, helium content and dew point of the gas, and metal flow rate. Superheat temperatures of from about 150° F. (66° C.) to 200° F. (93° C.) are preferred. Nozzle diameters of about 0.07 in. (1.8 mm) to 0.12 in. (3.0 mm) are preferred depending on the alloy. The gas stream used herein was a helium nitrogen mixture containing 74 to 87 vol. % helium. The metal flow rate ranged from about 0.8 lb/min (0.36 kg/min) to 4.0 lb/min (1.81 kg/min). The oxygen content of the L1<sub>2</sub> aluminum alloy powders was observed to consistently decrease as a run progressed. This is suggested to be the result of the oxygen gettering capability of the aluminum powder in a closed system. The dew point of the gas was controlled to minimize hydrogen content of the powder. Dew points in the gases used in the examples ranged from -10° F. (-23° C.) to -110° F. (-79° C.).

The powder is then classified by sieving process 290 to create classified powder 300. Sieving of powder is performed under an inert environment to minimize oxygen and hydrogen pickup from the environment. While the yield of minus 450 mesh powder is extremely high (95%), there are always larger particle sizes, flakes and ligaments that are removed by the sieving. Sieving also ensures a narrow size distribution and provides a more uniform powder size. Sieving also ensures that flaw sizes cannot be greater than minus 450 mesh which will be required for nondestructive inspection of the final product.

Processing parameters of exemplary gas atomization runs are listed in Table 1.

fifty gas atomization runs were performed to produce the inventive powder with finer powder size, finer size distribution, spherical shape, and lower oxygen and hydrogen contents. Processing parameters of some exemplary gas atomization runs are listed in Table 1. It is suggested that the observed decrease in oxygen content is attributed to oxygen gettering by the powder as the runs progressed.

Inventive L1<sub>2</sub> aluminum alloy powder was produced with over 95% yield of minus 450 mesh (30 microns) which includes powder from about 1 micron to about 30 microns. The average powder size was about 10 microns to about 15 microns. As noted above, finer powder size is preferred for higher mechanical properties. Finer powders have finer cellular microstructures. As a result, finer cell sizes lead to finer grain size by fragmentation and coalescence of cells during powder consolidation. Finer grain sizes produce higher yield strength through the Hall-Petch strengthening model where yield strength varies inversely as the square root of the grain size. It is preferred to use powder with an average particle size of 10-15 microns. Powders with a powder size less than 10-15 microns can be more challenging to handle due to the larger surface area of the powder. Powders with sizes larger than 10-15 microns will result in larger cell sizes in the consolidated product which, in turn, will lead to larger grain sizes and lower yield strengths.

Powders with narrow size distributions are preferred. Narrower powder size distributions produce product microstructures with more uniform grain size. Spherical powder was produced to provide higher apparent and tap densities which help in achieving 100% density in the consolidated product. Spherical shape is also an indication of cleaner and low oxygen content powder. Lower oxygen and lower hydrogen contents are important in producing material with high ductility and fracture toughness. Although it is beneficial to maintain low oxygen and hydrogen content in powder to achieve good mechanical properties, lower oxygen may interfere with sieving due to self sintering. An oxygen content of about 25 ppm to about 500 ppm is preferred to provide good ductility and fracture toughness without any sieving issue. Lower hydrogen is also preferred for improving ductility and fracture toughness. It is preferred to have about 25-200 ppm of hydrogen in atomized powder by controlling the dew point in the atomization chamber. Hydrogen in the powder is further reduced by heating the powder in vacuum. Lower hydrogen in final product is preferred to achieve good ductility and fracture toughness.

TABLE 1

Gas atomization parameters used for producing powder

| Run | Nozzle Diameter (in) | He Content (vol %) | Gas Pressure (psi) | Dew Point (° F.) | Charge Temperature (° F.) | Average Metal Flow Rate (lbs/min) | Oxygen Content (ppm) Start | Oxygen Content (ppm) End |
|-----|----------------------|--------------------|--------------------|------------------|---------------------------|-----------------------------------|----------------------------|--------------------------|
| 1   | 0.10                 | 79                 | 190                | <-58             | 2200                      | 2.8                               | 340                        | 35                       |
| 2   | 0.10                 | 83                 | 192                | -35              | 1635                      | 0.8                               | 772                        | 27                       |
| 3   | 0.09                 | 78                 | 190                | -10              | 2230                      | 1.4                               | 297                        | <0.01                    |
| 4   | 0.09                 | 85                 | 160                | -38              | 1845                      | 2.2                               | 22                         | 4.1                      |
| 5   | 0.10                 | 86                 | 207                | -88              | 1885                      | 3.3                               | 286                        | 208                      |
| 6   | 0.09                 | 86                 | 207                | -92              | 1915                      | 2.6                               | 145                        | 88                       |

The role of powder quality is extremely important to produce material with higher strength and ductility. Powder quality is determined by powder size, shape, size distribution, oxygen content, hydrogen content, and alloy chemistry. Over

65 The properties of five L1<sub>2</sub> aluminum alloy extruded bars are shown in Table 2. All samples exhibit tensile strengths over 100 ksi (690 MPa) and ductilities over 6%. Powder produced from the current invention was used for producing

## 13

these extrusions. The excellent tensile properties validate the inventive alloys and process described herein. The ultimate tensile strengths and yield strength of extruded bars of the current invention are significantly (30% to 150%) higher than aluminum alloys which are currently available including 7xxx, 6xxx and 2xxx series alloys. The strength and ductility (measured by elongation and reduction in area) observed in the present extrusions are directly related to the powder quality in terms of powder size, distribution, shape and micro-structure.

TABLE 2

| Tensile Properties of Extrusions of L1 <sub>2</sub> Aluminum Alloy Extrusions |                                |                     |               |                      |
|-------------------------------------------------------------------------------|--------------------------------|---------------------|---------------|----------------------|
| Material ID #                                                                 | Ultimate Tensile Strength, ksi | Yield Strength, ksi | Elongation, % | Reduction in Area, % |
| 1209                                                                          | 113.5                          | 103.2               | 7             | 15                   |
| 1210                                                                          | 113.5                          | 102                 | 6.5           | 12                   |
| 1213                                                                          | 116.3                          | 106.6               | 5.9           | 9                    |
| 1216                                                                          | 112.6                          | 102.3               | 6.5           | 10                   |
| 1222                                                                          | 116.6                          | 106.6               | 6.5           | 14.7                 |

Although the present invention has been described with reference to preferred embodiments, workers skilled in the art will recognize that changes may be made in form and detail without departing from the spirit and scope of the invention.

The invention claimed is:

1. An extruded high strength aluminum alloy containing L1<sub>2</sub> dispersoids, formed by the steps comprising:  
melting an aluminum alloy containing an L1<sub>2</sub> dispersoid forming element therein to a superheat temperature of from about 100° F. (38° C.) to about 300° F. (149° C.), wherein the L1<sub>2</sub> dispersoids comprise Al<sub>3</sub>X dispersoids wherein X is
  - (a) a first element consisting of about 0.1 to about 15.0 weight percent thulium; and at least one second element selected from the group consisting of about 0.1 to about 20.0 weight percent yttrium, about 0.05 to about 10.0 weight percent titanium, about 0.05 to about 10.0 weight percent hafnium, and about 0.05 to about 5.0 weight percent niobium;
  - (b) at least one third element selected from the group consisting of about 4 to about 25 weight percent silicon,

## 14

about 0.5 to about 3 weight percent lithium, about 0.2 to about 6 weight percent copper, about 3 to about 12 weight percent zinc, about 1 to about 12 weight percent nickel; and

(c) the balance substantially aluminum;  
forcing the melted alloy at a temperature of about 1600° F. (871° C.) to about 2200° F. (1204° C.) through a gas atomization nozzle with a diameter of from about 0.1 inches (254 microns) to about 0.2 inches (5.080 microns) under a helium pressure of about 160 psi (1.1 MPa) to about 207 psi (1.4 MPa) at a metal flow rate of from about 0.5 lb/min (0.23 kg/min) to about 25 lb/min (11.3 kg/min);

15 contacting the melted alloy leaving the nozzle with an inert gas stream to form liquid droplets, the inert gas stream having a pressure of about 50 psi (0.34 MPa) to about 750 psi (5.17 MPa);

cooling the droplets at a rate of at least 10<sup>3</sup>° C./second to form an alloy powder;  
sorting the powder to a mesh size of about minus 100 to about minus 635; and

extruding the powder to form an extruded aluminum alloy having tensile strength over 100 ksi (690 MPa) and ductilities over 6%.

20 2. The alloy of claim 1, wherein the gas atomization nozzle is a confined nozzle having a nozzle diameter of about 0.10 inch (2.54 mm).

30 3. The alloy of claim 1, wherein the inert gas is selected from at least one of argon, nitrogen and helium.

40 4. The alloy of claim 1, wherein oxygen is introduced during atomization such that the oxygen content of the powder is between 1 ppm and 2000 ppm and the hydrogen content is about 1 ppm to about 1000 ppm.

35 5. The alloy of claim 1, wherein the dew point of the gas stream is about minus 10° F. (minus 12.2° C.) to about minus 200° F. (minus 93° C.).

6. The alloy of claim 1, wherein the mean powder size is between 1 micron and 250 microns.

45 7. The alloy of claim 1, wherein the gas pressure to metal weight ratio is about 100 psi/lb (1.50 MPa/kg) to about 1500 psi/lbs (22.5 MPa/kg).

\* \* \* \* \*